

## UNITED STATES PATENT OFFICE

2,506,043

## PROCESS FOR OBTAINING TRANSPARENT EFFECTS ON REGENERATED CELLULOSE FIBERS

Paul Walter Steinlin, Basel, Switzerland, assignor to Aktiengesellschaft Cilander, Herisau, Switzerland

No Drawing. Application July 31, 1946, Serial No. 687,510. In Switzerland April 22, 1943

7 Claims. (Cl. 8—118)

1

The present application is in the nature of a continuation in part of my earlier copending application Serial No. 533,788, filed May 2, 1944, now abandoned.

Transparent fabrics, also known as organdies, have as a rule been made from pure cotton materials, in particular muslin, or, more rarely, voile or other fine fabrics, such as cambric, etc. Organdies of especially fine quality were made of natural silk.

The process hereafter described relates to the production of plain or patterned, smooth or crepe transparent fabrics from materials consisting of staple fibre made from regenerated cellulose alone or of staple fibre made from regenerated cellulose and cotton, or of mixed cotton and staple fibre made from regenerated cellulose.

Various experiments were made in the past to transform textiles of this kind by the ordinary methods used for cotton fabrics. However, even by varying and adapting working conditions, such as concentration of acids and alkaline swelling agents, and the duration of the procedure, it proved impossible to turn out marketable goods. Indeed the materials hitherto produced were horny, brittle and stiffened, and in no way suited for practical use. The present process, on the contrary, produces transparent fabrics which perfectly satisfy all requirements as to appearance, lustre, softness and durability, and show a high degree of transparency combined with a remarkable clearness of weave.

These effects are obtained by first treating the fabric with strong, hot alkali, then subjecting it to the action of strong, preferably cold sulphuric acid, and finally again treating it with strong alkali this time cold. The fabric can, eventually, be subjected to a treatment with alkaline or acid swelling agents either before or after.

The process is suited for fabrics made of pure staple fibre made from regenerated cellulose, or woven with cotton and staple fibre made from regenerated cellulose, and also for those woven with mixed staple fiber made from regenerated cellulose and cotton yarn. Naturally, materials in which any or all of the above combinations are present, either in plain or pattern weave, including of course applications with embroidery or Swiss dotted weave, can also be treated by my process.

It is advantageous to delubricate and bleach the fabric to be processed. Crude fabrics can, however, be treated in the same way. In this connection it should be borne in mind that, ac-

2

cording to the invention, this processing is suitable for use in any phase of pre-treatment.

My process can be used to advantage in combination with treatment by swelling agents. The order and manner in which these treatments are applied depend on the result desired.

In some cases a further improvement can be achieved by repeating the process wholly or in part.

10 Treatment with strong sulphuric acid is carried out with sulphuric acid of 40°-52° Bé. at temperatures ranging from -5° to +20° C. for at least 5 seconds.

15 Treatment with strong, cold alkali is carried out with an alkali of at least 15° Bé. at temperatures ranging from -5° to +25° C. for at least 5 seconds.

By hot alkali is understood a treatment according to the present process with hot alkali 20 solution of mercerizing strength, at a temperature of 25° C. or over, having a duration of 5 seconds or more.

It is advantageous to rinse and neutralize between acid and alkaline swelling treatments. Between 25 two consecutive alkaline treatments the question of rinsing and neutralizing is decided by the type of effect desired.

Patterned as well as plain transparent fabrics can be obtained with the present process by applying suitable reserves before the swelling treatment. For example imago effects can be achieved by printing with pigments, resulting in opaque non-transparent patterns. By this method it is possible, according to the type of process chosen,

35 to use pigment carriers proof against acid and alkaline swelling agents, such as gums or artificial resins, which result in local opaque effects, or non-acidproof thickening agents which produce stiffened transparent designs in which the effect of contrast is due to the pigmentation alone. It is moreover possible to introduce reserves during any phase of the transforming process so as to achieve, for example, a transparent effect and then, by rinsing and subsequent swelling and

40 shrinking, obtain the appearance of crepe. It is also possible to get intermediary effects by the imprint of swelling agents and subsequent treatment with hot alkali. The reserves can even be applied during various phases of the process in such a way that the transformed material shows untreated and swollen, that is shrunken and transparent areas one next to the other.

It is evident that by printing in colours or by the use of coloured reserves such effects can be obtained in various tints.

Fabrics submitted to the present process can be dyed either before or after treatment. In this way, according to the method of procedure, the most varied results can be obtained, such as plain transparent, or, according to the different affinity for the dye caused by different local treatment, shaded effects.

My process may be illustrated by means of a single example:

A singed, bleached and tentered fabric made from staple fibre made from regenerated cellulose is treated with NaOH of 30° Bé. at 50° C. for 8 seconds, rinsed, neutralized and dried. It is then subjected to the action of sulphuric acid of 45° Bé. at 15° C. for 7 seconds, neutralized and rinsed. Next comes a treatment with NaOH of 31° Bé. at 10° C. for 6 seconds. After neutralizing, rinsing and finishing in the usual way, a very fine staple fibre transparent fabric is obtained.

I claim:

1. A multiple step process for obtaining transparent effects upon a fabric consisting predominantly of regenerated cellulose staple fibers comprising treating said fabric with hot caustic soda of mercerizing strength at temperatures of the order of 50° C. for at least 5 seconds but not substantially more than 5 seconds, then treating said fabric with sulfuric acid of 40° to 52° Baumé at a temperature ranging from -5° to 20° C. for a period of time of the order of 5 to 7 seconds, and then treating said fabric with caustic soda of mercerizing strength at temperatures of -5° to 25° C. for at least 5 seconds but not substantially more than 5 seconds.

2. A multiple step process for obtaining transparent effects upon a fabric consisting predominantly of regenerated cellulose staple fibers comprising treating said fabric with hot caustic soda of mercerizing strength at temperatures of the order of 50° C. for at least 5 seconds but not substantially more than 5 seconds, removing free caustic soda from the fabric, then treating said fabric with sulfuric acid of 40° to 52° Baumé at a temperature ranging from -5° to 20° C. for a period of time of the order of 5 to 7 seconds, and then treating said fabric with caustic soda of mercerizing strength at temperatures of -5° to 25° C. for at least 5 seconds but not substantially more than 5 seconds.

3. A multiple step process for obtaining transparent effects upon a fabric consisting predominantly of regenerated cellulose staple fibers comprising treating said fabric with hot caustic soda of mercerizing strength at temperatures of the order of 50° C. for at least 5 seconds but not substantially more than 5 seconds, then treating said fabric with sulfuric acid of 40° to 52° Baumé at a temperature ranging from -5° to 20° C. for a period of time of the order of 5 to 7 seconds, removing free sulfuric acid from the fabric, and then treating said fabric with caustic soda of mercerizing strength at temperatures of -5° to 25° C. for at least 5 seconds but not substantially more than 5 seconds.

4. A multiple step process for obtaining transparent effects upon a fabric consisting predominantly of regenerated cellulose staple fibers comprising treating said fabric with hot caustic soda of mercerizing strength at temperatures of the order of 50° C. for at least 5 seconds but not sub-

stantially more than 5 seconds, washing and drying the fabric, then treating said fabric with sulfuric acid of 40° to 52° Baumé at a temperature ranging from -5° to 20° C. for a period of time of the order of 5 to 7 seconds, and then treating said fabric with caustic soda of mercerizing strength at temperatures of -5° to 25° C. for at least 5 seconds but not substantially more than 5 seconds.

5. A multiple step process for obtaining transparent effects upon a fabric consisting predominantly of regenerated cellulose staple fibers comprising treating said fabric with hot caustic soda of mercerizing strength at temperatures of the order of 50° C. for at least 5 seconds but not substantially more than 5 seconds, then treating said fabric with sulfuric acid of 40° to 52° Baumé at a temperature ranging from -5° to 20° C. for a period of time of the order of 5 to 7 seconds, 15 washing and drying the fabric, and then treating said fabric with caustic soda of mercerizing strength at temperatures of -5° to 25° C. for at least 5 seconds but not substantially more than 5 seconds.

20 6. A multiple step process for obtaining transparent effects upon a fabric consisting predominantly of regenerated cellulose staple fibers comprising treating said fabric with caustic soda of the order of 30° Baumé at a temperature of the order of 50° C. for a period of time of the order of 5 to 8 seconds, then treating said fabric with sulfuric acid of the order of 45° Baumé at a temperature of the order of 15° C. for a period of time of the order of 7 seconds, and then treating said fabric with caustic soda of the order of 31° Baumé at a temperature of the order of 10° C. for a period of time of the order of 6 seconds.

25 7. A multiple step process for obtaining transparent effects upon a fabric consisting predominantly of regenerated cellulose staple fibers comprising treating said fabric with caustic soda of the order of 30° Baumé at a temperature of the order of 50° C. for a period of time of the order of 8 seconds, rinsing, neutralizing, and drying the fabric, then treating said fabric with sulfuric acid of the order of 45° Baumé at a temperature of the order of 15° C. for a period of time of the order of 7 seconds, neutralizing and rinsing the fabric, and then treating said fabric with caustic soda of the order of 31° Baumé at a temperature of the order of 10° C. for a period of time of the order of 6 seconds.

PAUL WALTER STEINLIN.

#### REFERENCES CITED

The following references are of record in the file of this patent:

#### UNITED STATES PATENTS

| Number    | Name          | Date          |
|-----------|---------------|---------------|
| 1,439,517 | Heberlein     | Dec. 19, 1922 |
| 1,922,308 | Lilienfeld    | Aug. 15, 1933 |
| 1,989,100 | Lilienfeld    | Jan. 29, 1935 |
| 1,998,576 | Heberlein     | Apr. 23, 1935 |
| 2,202,200 | Haller et al. | May 28, 1940  |

#### FOREIGN PATENTS

| Number  | Country       | Date          |
|---------|---------------|---------------|
| 323,175 | Great Britain | Jan. 2, 1930  |
| 337,713 | Italy         | Mar. 11, 1936 |